

## UNITED STATES PATENT OFFICE

EDWARD C. BURDICK, OF MIDLAND, MICHIGAN, ASSIGNOR TO THE DOW CHEMICAL COMPANY, OF MIDLAND, MICHIGAN, A CORPORATION OF MICHIGAN

## LIGHT-METAL ALLOY AND METHOD OF MAKING SAME

No Drawing. Application filed December 11, 1924. Serial No. 755,166.

The constitution and method of making certain alloys of manganese with magnesium in which the magnesium largely predominates are disclosed in Patent No. 1,377,374 issued to W. R. Veazey May 10, 1921, and in a companion patent to the same inventor viz: No. 1,334,193, dated March 16, 1920, there is disclosed a ternary alloy of specific composition in which manganese is one and 10 copper the other ingredient added to the magnesium, such manganese and copper aggregating a relatively small percentage of the total.

I have found that a similarly relatively small percentage of manganese, with or without copper, materially improves for certain purposes the well known class of magnesium alloys in which aluminum is the principal alloying element.

20 The present invention then consists of the new alloy product containing magnesium and aluminum in approximately the proportions stated and in addition thereto a relatively small percentage of manganese or copper and 25 manganese. The invention also comprehends the steps involved in the making of such alloys, all as hereinafter fully described and particularly set forth in the claims, it being understood that the following description 30 sets forth but several of the various ways in which the invention may be carried out.

Magnesium alloys containing not less than 35 80 per cent. and not more than 99.5 per cent. of magnesium and not more than 20 per cent. or less than 0.5 per cent. of aluminum, are described in Patent No. 965,485 issued to G. Pistor et al., July 26, 1910, and the specific proportions illustrated in the example given 40 in this patent viz. 92 per cent. of magnesium and 8 per cent. of aluminum, have been found for many purposes most satisfactory. I have discovered, however, that the addition of manganese in an amount less than one per cent exercises a beneficial influence on an 45 alloy of this type, particularly as to the grain structure of castings made therefrom, as well as in other physical characteristics. Even a more marked improvement is effected where 50 copper in approximately the same small

amount is added to the alloy along with such manganese.

Where manganese alone is to be added to a magnesium-aluminum alloy of the type described, I preferably employ the method disclosed in the aforesaid Patent No. 1,377,374. For example, a measured quantity of the magnesium-aluminum alloy is melted up and then a limited quantity of anhydrous manganese chloride ( $MnCl_2$ ) is added thereto. 55 A flux of slightly greater specific gravity than the molten magnesium metal and having a sufficient surface tension to cause it to form a film thereover and thus prevent exposure of the metal to the atmosphere is 60 used in the crucible or melting pot, and when the anhydrous manganese chloride is added this flux is pushed aside for the purpose of permitting the chloride to come directly into contact with the molten metal. The chloride 65 is thenceupon immediately reduced and the resultant metallic manganese subject to certain losses, becomes alloyed with the magnesium and aluminum. The addition of manganese chloride calculated to provide 70 0.5 per cent of manganese in the resultant alloy will give, as a matter of fact, an alloy containing approximately 0.2 per cent.

Where in addition to such small percentage of manganese a corresponding small percentage of copper is to be added so as to make a magnesium-aluminum-copper-manganese alloy, this may be accomplished either by adding to a measured quantity of the magnesium-aluminum base in molten condition 75 the proper small amount of cupro-manganese or by first adding such cupro-manganese to the molten magnesium alone, and then adding aluminum to the resultant magnesium-copper-manganese alloy. Cupro-manganese is a known alloy of the two metals involved ordinarily containing seven parts of copper to three parts of manganese, and when added in the proportion of one per cent to magnesium alone or to a previously 80 prepared magnesium-aluminum alloy of the type hereinbefore referred to, will produce a resultant alloy in which the amount of manganese is slightly reduced as a result of 85 apparently unavoidable losses, so that the 90 95

final product will show an analysis of approximately 0.2 per cent of manganese and approximately 0.7 per cent copper.

As a specific illustration of the making of a magnesium-aluminum-copper-manganese alloy in accordance with the foregoing general procedure, I take twenty pounds of a magnesium-copper-manganese alloy, made as just described, and containing 0.70 per cent of copper and 0.20 per cent of manganese and add thereto three successive quantities of six ounces each of aluminum. The analyses of the resultant quaternary alloys will then show aluminum in approximately 15 the following amount viz., 1.84 per cent, 3.84 per cent and 5.97 per cent, respectively, the relative proportions of copper and manganese remaining substantially unchanged from the figures just given. Bars cast from 20 such quaternary alloy and machined for test purposes show a Brinnell hardness of slightly less than 70 and yield points successively increasing with the amount of aluminum present from approximately 25 9000 pounds for the 1.84 per cent aluminum contents to approximately 11,000 pounds for the 3.84 per cent aluminum content, and approximately 12,000 pounds for the 5.97 per cent aluminum content.

30 An alloy similar to the foregoing but containing an aluminum content of between 8 and 8.5 per cent shows a somewhat increased Brinnell hardness and a considerably increased yield point viz. approximately 15,000 35 pounds. As previously indicated, for most purposes this may be regarded as the alloy 95 composition of the type described herein as new.

Other modes of applying the principle of 40 my invention may be employed instead of the one explained, change being made as regards the composition and method herein disclosed, provided the ingredients or steps stated by any of the following claims or the 45 equivalent of such stated ingredients or steps 100 be employed.

I therefore particularly point out and distinctly claim as my invention:

1. The method of making an aluminum-50 copper-manganese alloy of magnesium, which comprises forming an alloy of magnesium and aluminum in which the magnesium largely predominates, and incorporating in such alloy in molten state, a cupro- 55 manganese alloy.

2. As a new product, an alloy containing magnesium in excess of eighty per cent., manganese in an amount not exceeding five-tenths of one per cent., and the balance principally aluminum with a relatively small amount of copper.

3. As a new product, a magnesium-aluminum-copper-manganese alloy wherein the magnesium is in excess of eighty per cent., 65 the copper not exceeding two per cent., the 105

manganese in amount not exceeding five-tenths of one per cent., and the aluminum exceeds the copper.

4. As a new product, a magnesium-aluminum-copper-manganese alloy containing in excess of ninety per cent. magnesium, 70 from two to eight and one-half per cent. aluminum and approximately one per cent. of cupro-manganese.

5. As a new product, a magnesium-aluminum-copper-manganese alloy consisting of approximately ninety three per cent. magnesium, six per cent. aluminum, seven-tenths of one per cent. of copper, and one-quarter of one per cent. of manganese.

Signed by me this 5th day of December, 1924.

EDWARD C. BURDICK.

85

90

95

100

105

110

115

120

125

130